

July 6, 1971

A. GUZZI ET AL  
SILVER HALIDE EMULSION CONTAINING  
NAPHTHAMIDE PHOTOGRAPHIC COUPLERS  
Filed Jan. 31, 1968

3,591,384

FIG. 1



FIG. 2



INVENTORS

ALBERTO GUZZI  
REMO MAGAGNOLI  
BY  
Carpenter, Kinney & Coulter  
ATTORNEYS

1

3,591,384

SILVER HALIDE EMULSION CONTAINING  
NAPHTHAMIDE PHOTOGRAPHIC COUPLERS  
Alberto Guzzi and Remo Magagnoli, Ferrania, Italy, as  
signors to Societa per Azioni Ferrania, Milan, Italy  
Filed Jan. 31, 1968, Ser. No. 701,995

Claims priority, application Italy, Feb. 15, 1967,

34,846/67

Int. Cl. G03c 1/40  
U.S. Cl. 96—100

6 Claims 10

## ABSTRACT OF THE DISCLOSURE

This invention relates to compounds useful as photographic couplers having the general formula:



wherein X is alkyl, Y is either carbonyl or sulfonyl, R is alkyl having from 5 to 20 carbon atoms and Z is hydrogen or halogen. The invention also relates to the use of the abovementioned compounds in photographic emulsions.

This invention relates to a class of couplers capable of forming stable cyan or blue-green dyes by color development in color photographic materials.

In the production of colored images by the color development of silver halide emulsion layers in a multi-layer film construction the image formed after light exposure of the reducible silver salts is developed in the presence of a coupler, i.e. a compound which reacts with the oxidation products of the color developer to form a dye. Cyan images are generally obtained by the formation of an indophenol dye from a 1-hydroxy-2-naphthamide coupler.

One important requirement of color couplers used in color photography is the ability to resist bleeding or migration through and outside of the photographic emulsion layers in which they are contained. An effective means for solving the migration problem is provided by the dispersed coupler method, in which the coupler is dissolved in high boiling organic solvents, such as tricresyl phosphate or dibutyl phthalate, and the resulting solution is intimately dispersed throughout the silver halide emulsion. To obtain the best results in terms of the dispersion and photographic efficiency the solution of coupler in the organic solvent should be highly concentrated. Couplers which are highly soluble in or miscible with the organic solvent are therefore commonly selected for use in dispersed coupler systems. In general, couplers having a relatively low melting point are quite soluble in such organic solvents. However, it is also desirable to select couplers which produce dyes having good stability to light, heat

2

and moisture and having good spectral characteristics, particularly low secondary absorptions.

It is an object of this invention to provide a new class of outstanding cyan couplers and photographic emulsions incorporating such couplers.

The cyan couplers of this invention have the formula:



wherein X is alkyl, preferably a lower alkyl (C<sub>1</sub>—C<sub>6</sub>), Y is either carbonyl or sulfonyl, R is C<sub>5</sub>—C<sub>20</sub> alkyl, and Z is hydrogen or halogen, preferably chlorine or bromine. These couplers are easily obtained in a very high purity by methods described later.

Illustrative couplers are as follows:



(1)



(2)



(3)



(4)

Table I shows some analytical data of these illustrative couplers, the analyses being made after only one crystallization of the raw reaction product. Included are their desirable melting points. Their high degree of solubility in organic solvents normally used for dispersing couplers in a gelatin emulsion permits the use of a solvent/coupler ratio far lower than 1.0 without any noticeable decrease in yield of dye formed by normal color development procedures. For example, coupler (1) can be incorporated into a photographic emulsion with 1 part dibutyl phthalate containing 4 parts of coupler.

TABLE I

| Coupler No. | Melting point (° F.)         | C, percent |       | H, percent |       | N, percent |       | Cl, percent |       | —OH, percent content found | Crystallization solvent |
|-------------|------------------------------|------------|-------|------------|-------|------------|-------|-------------|-------|----------------------------|-------------------------|
|             |                              | Found      | Calc. | Found      | Calc. | Found      | Calc. | Found       | Calc. |                            |                         |
| 1.....      | 215.6-219.2<br>(102-104° C.) | 78.46      | 78.39 | 8.28       | 8.11  | 3.00       | 3.04  | .....       | ..... | 99.27                      | Ethanol.                |
| 2.....      | 149.0-150.8<br>(65-66° C.)   | 72.55      | 72.9  | 7.25       | 7.3   | .....      | ..... | 7.16        | 7.17  | 98.81                      | Heptane.                |
| 3.....      | 208.4-210.2<br>(98-99° C.)   | .....      | ..... | .....      | ..... | .....      | ..... | .....       | ..... | 99.41                      | Acetic acid.            |
| 4.....      | 240.8-242.6<br>(116-117° C.) | .....      | ..... | .....      | ..... | 5.86       | 5.90  | .....       | ..... | 98.44                      | Do.                     |

In addition to the above-mentioned characteristics the claimed couplers react with N,N-dialkyl-p-phenylenediamine during color development to provide dyes which are particularly stable to light, heat and moisture. For example, if one of these couplers is dissolved in dibutyl phthalate, dispersed in a photographic emulsion, coated onto a transparent support, exposed and developed with diethyl-p-phenylenediamine, the resultant color shows no noticeable change in either color density or hue after exposure to a xenon lamp for 10 hours. Coated samples prepared in similar manner were exposed through a scale of decreasing densities, i.e. grey scale, and developed in color developer with excellent sensitometric results, even after storage for 2 hours at a temperature of 194.0° F. (90° C.) and a relative humidity of 75%. In FIG. 1 curve A is the sensitometric curve (read in red light) for coupler (1) and curve B is the sensitometric curve for coupler (1) after 24 hours storage under the above-mentioned conditions. These curves show the excellent stability of dyes prepared from the couplers of this invention.

The spectral absorption of the cyan dyes obtained from these couplers and N,N-dialkyl-p-phenylenediamine developers make them particularly suitable for preparing color negative materials. Furthermore, they have a low absorption in the green portion of the spectrum, which is very desirable. In FIG. 2 an illustrative comparison of the spectral absorption of N,N-diethyl-p-phenylenediamine developed couplers in dibutyl phthalate, absorption curve A being that of abovementioned coupler (3) and absorption curve B being that of a coupler of the formula:



The coupler of curve B is a known coupler having some structural similarity to the couplers of this invention. From a comparison of curves A and B it is apparent that curve A represents lower absorption in the 500 and 600 millimicron region than curve B.

The couplers of the present invention can be prepared by reacting the suitable amines with 1-hydroxy-2-naphthoic acid or 1-hydroxy-4-halo-2-naphthoic acid derivatives, such as their phenyl esters. In particular, the preparations of some couplers of said class were carried out in the following way:

(a) PREPARATION OF 4-METHYLLAUROPHENONE

Into a 500 ml. flask containing a suspension of 59 g. of  $AlCl_3$  in 168 ml. of dry toluene, 69.2 g. of lauroyl chloride were rather quickly introduced. The temperature rose to 140.0° F. (60° C.). The mixture was kept under stirring at a temperature of 176.0° F. (80° C.) for 22 hours, then was poured with vigorous stirring into 1000 ml. of water and 66.5 ml. of concentrated hydrochloric acid. After about one hour the organic layer was removed and washed, first with a 1%  $Na_2CO_3$  solution and then with water. The toluene solution was then dried with calcium chloride, and the solvent was removed under vacuum. The residue, consisting of a readily solidifying oil, was crystallized from ethanol. Yield: 58.8 g. (67%). M.P.: 113.0–115.5° F. (45°–46.5° C.).

Analysis.—Calculated for  $C_{19}H_{30}O$  (percent): C, 83.57; H, 10.94. Found (percent): C, 83.27; H, 10.94.

(b) PREPARATION OF 3-NITRO-4-METHYL-LAUROPHENONE

In a beaker provided with stirrer and thermometer, was placed 190 ml. of  $HNO_3$  (d=1.52) and then 69.9 g. of 4-methyllaurophenone was added in increments. The operation was carried out as rapidly as possible while

maintaining the reaction temperature below 44.6° F. (7° C.). After completion of the ketone addition the mixture was stirred for an additional 5 minutes and then the mixture was added dropwise into one liter of ice water. The precipitated product was filtered off and thoroughly washed with water, then allowed to dry in the air. By crystallization from methanol 86.4 g. (70%) of the nitro derivative with M.P.: 122.0–123.8° F. (50°–51° C.) was obtained.

(c) PREPARATION OF 3-AMINO-4-METHYL-LAUROPHENONE

56.4 g. of 3-nitro-4-methyllaurophenone was dissolved in a boiling mixture of 530 ml. of 90% acetic acid and 260 ml. of ethanol. Then 106 g. of iron powder was slowly added. After completion of the addition boiling was continued for about 30 minutes, after which the ferrous slime was hot filtered and the filtrate was poured with stirring into 17.5 ml. of water. The amine which separated was filtered off and thoroughly washed with water. Yield of raw product: 48.6 g. By crystallizing the raw product from 485 ml. of ethanol and decolorizing with charcoal, 41.5 g. (81.2%) of product having a M.P. of 167.0°–170.6° F. (75°–77° C.) was obtained.

Analysis.—Calculated for  $C_{19}H_{31}NO$  (percent): N, 4.84. Found (percent): N, 4.65; —NH<sub>2</sub> content, 100.00.

(d) PREPARATION OF 1-HYDROXY-2-(2'-METHYL-5'-LAUROYL)NAPHTHANILIDE (COUPLER 1)

In a Claisen flask arranged for distillation under vacuum a mixture of 63.6 g. of 3-amino-4-methyllaurophenone and 63.6 g. of phenyl 1-hydroxy-2-naphthoate was melted. At this point vacuum was applied in order to remove the phenol which was liberated as the reaction continued. After about half an hour the amount of distilled phenol was 22 g. (theory: 22.6 g.). The residue was crystallized from ethanol. Yield of coupler: 91.5 g.

(e) PREPARATION OF 1-HYDROXY-4-CHLORO-2-2'-METHYL-5'-LAUROYL)NAPHTHANILIDE (COUPLER 2)

By working in the same way as described for the coupler 1 and employing an equivalent amount of phenyl 1-hydroxy-4-chloro-2-naphthoate instead of phenyl 1-hydroxy-2-naphthoate 86 g. of coupler was obtained after crystallization from heptane.

(f) PREPARATION OF p-TOLYL CETYL SULFONE

50 Into a reaction flask 75 g. of sodium p-toluenesulfonate tetrahydrate, 300 ml. of ethanol and 91.5 g. of cetyl bromide were introduced. The mixture was heated at reflux on a water bath for 24 hours and was then diluted with 1 liter of water. A white precipitate was obtained which, after being filtered, washed and dried, was purified by crystallization from ethanol. Yield: 82.1 g. M.P.: 154.4–156.2° F. (68–69° C.).

Analysis.—Calculated for  $C_{23}H_{40}O_2S$  (percent): C, 72.57; H, 10.5; S, 8.4. Found (percent): C, 72.36; H, 10.4; S, 8.28.

(g) PREPARATION OF 3-NITRO-4-METHYL-PHENYL CETYL SULFONE

65 It was obtained in a way similar to the 3-nitro-4-methyl-laurophenone by using 112 ml. of fuming  $HNO_3$  for 56.8 g. of p-tolyl-cetyl sulfone. Yield: 55.2 g. (from ethanol) M.P.: 161.6°–163.4° F. (72–73° C.).

(h) PREPARATION OF 3-AMINO-4-METHYL-PHENYL ACETYL SULFONE

Prepared in a way similar to the 3-amino-4-methyl-laurophenone, it was crystallized from ethanol. M.P.: 140.0°–141.8° F. (60°–61° C.).

Analysis.—NH<sub>2</sub> content 98.27%.

(i) PREPARATION OF 1-HYDROXY-2-(2'-METHYL-5'-CETYLSULFONYL) - NAPHTHANILIDE (COUPLER 3)

By following the same procedure as with coupler (1), 47.3 g. of 3-amino-4-methylphenyl cetyl sulfone was reacted with 34.7 g. of phenyl 1-hydroxy-2-naphthoate. 59.2 g. of coupler (3) was obtained.

(j) PREPARATION OF 1-HYDROXY-4-CHLORO-2-(2'-METHYL-5'-CETYLSULFONYL)-NAPHTHANILIDE (COUPLER 4)

The product was obtained by procedures similar to those used in the preceding examples from 39.5 g. of 3-amino-4-methylphenyl cetyl sulfone and 32.8 g. of phenyl 1-hydroxy-4-chloro-2-naphthoate. Yield was 43 grams.

(k) PREPARATION OF 1-HYDROXY-2-(2'-METHYL-5'-DECYLSULFONYL)NAPHTHANILIDE

Obtained by a synthesis similar to that of the coupler (3), using decyl bromide instead of cetyl bromide.

The properties of the intermediates are the following:

TABLE II

| Intermediate                       | M.p., ° F.                  | Crystallization solvent |
|------------------------------------|-----------------------------|-------------------------|
| p-Tolyldecylsulfone                | 125.6-129.2<br>(52°-54° C.) | Ethanol.                |
| 3-nitro-2-methylphenyldecylsulfone | 114.8-118.4<br>(46°-48° C.) | Ligroin.                |
| 3-amino-4-methylphenyldecylsulfone | 68.0<br>(<20° C.)           |                         |

The coupled was obtained by the reaction of the raw amine with phenyl 1-hydroxy-2-naphthoate and, after crystallization from ethanol, the M.P. was 273.2-277.5° F. (134°-136.5° C.).

Analysis—OH/content=96.87%.

Example 1

2 grams of coupler (1) was dissolved in a mixture consisting of 0.5 ml. of dibutyl phthalate and 12 ml. of ethyl acetate by heating on a boiling water bath. The resulting clear solution was poured into 40 ml. of 4% gelatin containing 4 ml. of 10% sodium tetradecyl sulfate solution. At a temperature of about 104.0° F. (40° C.) the mixture was dispersed in a homogenizer. The dispersion thus obtained was added to 200 g. of silver halide photographic emulsion sensitized to red light. The thus modified emulsion was spread on a transparent support, dried and exposed through an original. By chromogenic development in a N,N-diethyl-p-phenylenediamine developer, a negative blue-green colored image was obtained. The stable blue-green dye forming the image had an absorption peak at 688 m $\mu$ .

Example 2

A dispersion of the following formulation:

Coupler (3)—2 grams  
Dibutyl phthalate—4 ml.  
Ethyl acetate—12 ml.  
4% gelatin—40 ml.  
10% sodium tetradecyl sulfate solution—4 ml.

was added to 200 grams of a negative-type silver halide emulsion, sensitized to red light. The thus modified emulsion was spread onto a transparent support and dried. The photosensitive material thus obtained was exposed through an original and developed in a color developer of the following formulation:

|                                                     | Grams |
|-----------------------------------------------------|-------|
| Hydroxylamine hydrochloride                         | 1     |
| Diethyl-p-phenylenediamine sulfate                  | 2.8   |
| Sodium tripolyphosphate                             | 2     |
| Anhydrous sodium carbonate                          | 65    |
| Anhydrous sodium sulfite                            | 25    |
| Potassium bromide                                   | 1.2   |
| Water to make 1000 ml.<br>(pH 10.8-8.11 with NaOH). |       |

After the usual steps of bleaching, fixing and washing, a blue-green colored negative image of the original was obtained. The absorption curve of the blue-green dye forming the image is the same as curve A in FIG. 2. The absorption peak of the dye lies at 697-702 m $\mu$ .

Various other embodiments of the present invention will be apparent to those skilled in the art without departing from the scope thereof.

The embodiments of the invention in which an exclusive property or privilege is claimed are defined as follows:

1. A silver halide photographic emulsion containing dispersed therein at least one compound of the general formula:



wherein X is lower alkyl, Y is carbonyl or sulfonyl, R is an alkyl group having from 5 to 20 carbon atoms, and Z is hydrogen or halogen.

2. A photographic element having at least one layer comprising the emulsion of claim 1.

3. The emulsion of claim 1 wherein said compound has the formula



4. The emulsion of claim 1 wherein said compound has the formula



5. The emulsion of claim 1 wherein said compound has the formula



6. The emulsion of claim 1 wherein said compound has the formula



References Cited

UNITED STATES PATENTS

70 3,459,552 8/1969 Yoshida et al. ----- 96-100  
J. TRAVIS BROWN, Primary Examiner

U.S. Cl. X.R.

UNITED STATES PATENT OFFICE  
CERTIFICATE OF CORRECTION

Patent No. 3,591,384 Dated July 6, 1971

Inventor(s) Alberto Guzzi and Remo Magagnoli

It is certified that error appears in the above-identified patent and that said Letters Patent are hereby corrected as shown below:

Column 3, line 14, "2 hours" should read -- 24 hours --;

Column 4, line 33, "1-hydroxy-2-naphthorate" should read -- 1-hydroxy-2-naphthoate --;

Column 4, line 40, "2'-methyl" (etc.) should read -- (2'-methyl -- (etc.);

Column 4, line 70, "acetyl" should read -- cetyl --;

Column 5, line 31, "coupled", should read -- coupler --;

Column 6, line 15,



should read --



Signed and sealed this 26th day of September 1972.

(SEAL)

Attest:

EDWARD M. FLETCHER, JR.  
Attesting Officer

ROBERT GOTTSCHALK  
Commissioner of Patents